

## AGE HARDENING AUSTENITIC STEEL

Reinhold Schempp, Clay, Peter Payson, New York, and Joe Gin-Young Chow, Long Island City, N. Y., assignors to Crucible Steel Company of America, New York, N. Y., a corporation of New Jersey

No Drawing. Application February 18, 1953,  
Serial No. 337,688

2 Claims. (Cl. 75—128)

This invention pertains to improvements in austenitic steels, and provides a relatively high carbon, high phosphorus, steel of this type which is age hardenable to a minimum of "C" 32 and up to about "C" 50 Rockwell depending upon the analysis, and which is further characterized by high strength and corrosion resistance at both room and elevated temperatures.

This application is a continuation-in-part of our copending application Serial No. 294,260, filed June 18, 1952, now Patent No. 2,686,116, issued August 10, 1954.

Objects of this invention are: to provide austenitic age hardenable steels which are useful for applications where high strength at room temperature combined with low magnetic permeability are required, as for studs, gears, crankshafts, and so on, in non-magnetic power plants of submarines; for retainer rings on rotors of electric generators; and so forth; also where hardness and resistance to softening at elevated temperatures upward of 1300° F. combined with good resistance to oxidation and corrosion at such temperatures are required, particularly in combustion products of leaded gasoline, as for automotive exhaust valves, valve seats, and similar parts; and finally, where high strength at temperatures upward of 1100° F. is required together with resistance to oxidation at these temperatures, as for steam power plant and gas turbine parts.

Another object of this invention is to provide an austenitic steel which is hardenable to a minimum of "C" 32 Rockwell, or 300 Brinell.

Another object of this invention is to provide an austenitic age hardenable steel which can be hardened to a minimum of "C" 32 Rockwell by use of a solution temperature no higher than 2200° F.

In a copending application of one of the present inventors, Serial No. 222,736, filed April 20, 1951, there are disclosed austenitic steels containing: 0.4 to 1.5% carbon; 12 to 30% chromium; 0 to 25% nickel 0.1 to 25% manganese; the combined nickel and manganese content comprising 8 to 28%; 0 to 5% silicon; balance substantially iron, which are age hardenable to at least "C" 32 Rockwell by a heat treatment consisting of solution treating at about 2300° F. and quenching, and thereupon aging at about 1300° F. An appreciable deterrent to the use of such hardened steel is the very high solution temperature required. Even with modern furnace equipment and design it is not easy to heat treat large quantities of parts at such high temperatures, particularly if the parts are sizeable. Furthermore, the solidus temperature of such steel is not much above 2350° F. Thus the solution temperature is dangerously close to the temperature at which the steel begins to melt, and there is considerable hazard therefore in the handling of such steel at the temperature required for proper solution treatment for the desired hardening.

Now we have discovered that by introducing about 0.15 to 0.45% phosphorus into steel of approximately the composition given above, the necessary solution temperature

can be lowered appreciably from the undesirably high temperature required for the steel in the absence of this phosphorus content. Depending on the phosphorus content, the necessary solution temperature can be lowered to about 2150° F. with moderate amounts, say about 0.20%, and even to 1950° F. when amounts of about 0.4% phosphorus are used.

We have discovered, however, that the addition of high phosphorus within the above range, necessitates a critical balancing and proportioning of the elements carbon, nickel, manganese and chromium in order to assure that the steel will have the requisite minimum age hardenability of the "C" 32 Rockwell.

That the minimum carbon and phosphorus contents are particularly critical in this respect is shown by the data contained in the following Tables I to IV, inc.

Table I

### LOW CARBON AUSTENITIC STEELS WITH PHOSPHORUS

[Solution treated at 2150° F. and 2300° F. and water quenched; aged at 1200°, 1300°, 1400° F. for 16 hours.]

| Bar       | C   | Mn  | P   | Si  | Ni   | Cr   | N   | Bal. |
|-----------|-----|-----|-----|-----|------|------|-----|------|
| 3915..... | .05 | 1.5 | .10 | .40 | 11.1 | 18.0 | .26 | Fe   |
| 3918..... | .05 | 1.4 | .27 | .37 | 11.3 | 18.8 | .21 | Fe   |

| 30                           | "C" Rockwell Hardness |           |           |           |
|------------------------------|-----------------------|-----------|-----------|-----------|
|                              | Bar 3915              |           | Bar 3918  |           |
|                              | 2,150° F.             | 2,300° F. | 2,150° F. | 2,300° F. |
| As solution Treated.....     | 8                     | 7         | 6         | 6         |
| Aged 1,200° F.—16 hours..... | 8                     | 7         | 8         | 8         |
| Aged 1,300° F.—16 hours..... | 8                     | 7         | 20        | 21        |
| Aged 1,400° F.—16 hours..... | 9                     | 8         | 19        | 19        |

Evidently although some hardening is attainable in the above low carbon steel containing about 0.27% P, the attainable hardness is considered insufficient for the parts we wish to make from a hardenable austenitic steel. However, when higher carbon is used in the steel along with high phosphorus the desired hardness of over "C" 32 Rockwell can be obtained as shown in Table II.

Table II

### EFFECT OF C ON ATTAINABLE HARDNESS IN AUSTENITIC C-Mn-Ni-Cr STEELS CONTAINING PHOSPHORUS

[Specimens solution treated at 2150° F., water quenched, and aged at 1250° for 16 hours.]

| 55        | Bar | Analysis Percent—Balance Fe |     |     |      |      |     |    | "C" Rockwell Hardness |             |
|-----------|-----|-----------------------------|-----|-----|------|------|-----|----|-----------------------|-------------|
|           |     | C                           | Mn  | P   | Si   | Ni   | Cr  | N  | As Quenched           | After Aging |
| 3965..... | .24 | 9.1                         | .21 | .32 | 2.2  | 20.3 | .20 | 21 | 29                    |             |
| 3968..... | .37 | 9.8                         | .21 | .83 | 4.0  | 22.0 | .24 | 23 | 44                    |             |
| 3978..... | .56 | 9.0                         | .21 | .90 | 3.7  | 20.6 | .21 | 31 | 45                    |             |
| 3990..... | .20 | 5.1                         | .34 | .49 | 3.8  | 21.6 | .21 | 23 | 31                    |             |
| 3897..... | .34 | 4.9                         | .38 | .40 | 3.8  | 21.5 | .20 | 22 | 47                    |             |
| 3902..... | .49 | 5.1                         | .36 | .58 | 3.8  | 21.6 | .22 | 29 | 49                    |             |
| 4492..... | .23 | 1.4                         | .23 | .44 | 13.3 | 18.0 | .06 | 11 | 33                    |             |
| 4491..... | .28 | 3.2                         | .18 | .39 | 9.1  | 18.3 | .07 | 11 | 34                    |             |
| 4488..... | .24 | 3.2                         | .23 | .40 | 9.2  | 18.6 | .09 | 11 | 35                    |             |
| 4494..... | .27 | 1.2                         | .24 | .38 | 13.1 | 17.5 | .07 | 11 | 36                    |             |
| 4490..... | .32 | 3.4                         | .22 | .38 | 9.1  | 18.3 | .07 | 11 | 37                    |             |
| 4489..... | .25 | 3.5                         | .32 | .40 | 9.2  | 18.6 | .06 | 11 | 41                    |             |
| 4493..... | .26 | 1.3                         | .34 | .40 | 13.1 | 18.3 | .08 | 11 | 40                    |             |
| 4495..... | .28 | 1.4                         | .34 | .35 | 13.0 | 18.1 | .12 | 11 | 42                    |             |

The effect of phosphorus on the attainable hardness of the steel after a solution treatment at 2150° F. and aging at 1250° F. is shown in Table III and Table IV,

Table III

EFFECT OF PHOSPHORUS ON ATTAINABLE HARDNESS OF MEDIUM CARBON AUSTENITIC Mn-Ni-Cr STEELS  
[Specimens solution treated at 2150° F., water quenched, and aged at 1300° F. for 16 hours.]

| Bar  | Analysis Percent—Balance Fe |     |     |     |      |      | "C" Rockwell Hardness |             |             |
|------|-----------------------------|-----|-----|-----|------|------|-----------------------|-------------|-------------|
|      | C                           | Mn  | P   | Si  | Ni   | Cr   | N                     | As Quenched | After Aging |
| 3940 | .33                         | 3.2 | .13 | .44 | 9.4  | 18.6 | .05                   | 14          | 28          |
| 3946 | .32                         | 1.5 | .13 | .37 | 13.0 | 19.0 | .05                   | 13          | 26          |
| 3949 | .45                         | 1.4 | .12 | .33 | 13.0 | 18.7 | .06                   | 18          | 28          |
| 3941 | .36                         | 3.5 | .24 | .33 | 9.4  | 18.9 | .05                   | 15          | 38          |
| 3947 | .36                         | 1.4 | .24 | .22 | 13.0 | 18.8 | .04                   | 15          | 35          |
| 3950 | .49                         | 1.4 | .23 | .20 | 13.1 | 18.8 | .05                   | 19          | 35          |

Table IV

EFFECT OF PHOSPHORUS ON ATTAINABLE HARDNESS OF HIGH CARBON AUSTENITIC C-Mn-Ni-Cr STEELS  
[Specimens solution treated at 2150° F., water quenched, and aged at 1250° F. for 16 hours.]

| Bar  | Analysis Percent—Balance Fe |     |     |     |     |      | "C" Rockwell Hardness |             |             |
|------|-----------------------------|-----|-----|-----|-----|------|-----------------------|-------------|-------------|
|      | C                           | Mn  | P   | Si  | Ni  | Cr   | N                     | As Quenched | After Aging |
| 3821 | .61                         | 2.3 | .09 | .39 | 9.1 | 20.9 | .04                   | 23          | 28          |
| 3817 | .60                         | 4.7 | .20 | .50 | 3.8 | 21.2 | .04                   | 29          | 40          |
| 3819 | .61                         | 5.0 | .41 | .41 | 3.7 | 20.7 | .04                   | 28          | 48          |
| 3825 | .61                         | 1.4 | .44 | .39 | 9.8 | 21.0 | .15                   | 27          | 48          |

From the data of Tables II—IV, inc., it will be seen

plus manganese content may be lowered to about 9%, as evidenced by bar 3902.

The upper limit for carbon is established by forgeability, and for forgeable steels of the invention, is set at about 0.8%. For castings the carbon may range as high as about 1.5%. Thus, the broad range for carbon is about 0.2 to 1.5%, or about 0.2 to 0.8% for the forgeable analyses. The preferred range for the forgeable alloys is about 0.3 to 0.8%.

10 With increasing phosphorus, the forgeability of the steel likewise decreases, and therefore the upper limit is set at about 0.45% P for the wrought material. However, for cast material we may employ as high as 1% P. The lower limit is set at about 0.15% P to assure adequate age hardening.

Manganese may be present over the range of 0.5 to 15%, and nickel over the range of about 3 to 25%, the sum of these two being present within a broad range of 9 to 30%, and within a narrow range of about 12 to 30%.

20 As above noted, the broad range is applicable to analyses containing upwards of 0.3% carbon and the narrow range to analyses containing lower carbon contents down to about 0.2%.

25 As stated earlier, in the high carbon, Mn-Ni-Cr steels of the copending application it is necessary to solution treat at about 2300° F. in order to develop a hardness of "C" 32 Rockwell or higher in the steel after aging. When a minimum of about 0.15% phosphorus is in the steel, however, adequate hardness may be developed with solution treatments no higher than 2200° F., the higher the phosphorus, the lower the necessary solution temperature. This is illustrated by data in Table V.

Table V

EFFECT OF PHOSPHORUS ON THE SOLUTION TEMPERATURE NECESSARY FOR DEVELOPING ADEQUATE HARDNESS IN C-Mn-Ni-Cr AUSTENITIC STEEL  
[Specimens quenched from indicated solution temperature and aged at 1250° F. for 16 hours.]

| Bar  | Analysis Percent—Balance Fe |     |     |     |     |      |     |     | "C" Rockwell Hardness |      |             |      |             |      |
|------|-----------------------------|-----|-----|-----|-----|------|-----|-----|-----------------------|------|-------------|------|-------------|------|
|      | C                           | Mn  | P   | Si  | Ni  | Cr   | Mo  | N   | 1,900° F.             |      | 2,000° F.   |      | 2,150° F.   |      |
|      |                             |     |     |     |     |      |     |     | As Quenched           | Aged | As Quenched | Aged | As Quenched | Aged |
| 3832 | .48                         | 7.8 | .15 | .40 | 7.3 | 22.1 | 1.8 | .06 | 23                    | 23   | 21          | 23   | 21          | 32   |
| 3716 | .65                         | 4.8 | .19 | .19 | 3.8 | 20.6 | —   | .07 | 32                    | 33   | 32          | 35   | 28          | 43   |
| 3975 | .36                         | 5.0 | .21 | .58 | 3.8 | 21.4 | —   | .22 | —                     | —    | 25          | 37   | 22          | 43   |
| 3933 | .51                         | 7.5 | .23 | .47 | 7.4 | 22.2 | 1.8 | .05 | 23                    | 29   | 23          | 32   | 23          | 40   |
| 3897 | .34                         | 4.9 | .33 | .40 | 3.8 | 21.5 | —   | .20 | 31                    | 37   | 28          | 42   | 21          | 47   |
| 3807 | .35                         | 1.4 | .38 | .33 | 9.3 | 21.1 | —   | .26 | 27                    | 39   | 27          | 43   | 22          | 47   |
| 3934 | .53                         | 7.5 | .41 | .36 | 7.3 | 21.5 | 1.7 | .07 | 27                    | 35   | 26          | 38   | 24          | 47   |
| 3825 | .61                         | 1.4 | .44 | .39 | 9.8 | 21.0 | —   | .15 | 26                    | 40   | 27          | 41   | 26          | 48   |

that all analyses containing at least 0.3% carbon together with at least 0.15% phosphorus, age harden adequately, i. e., to a minimum of "C" 32 Rockwell. On the other hand, analyses containing carbon below 0.3% and down to about 0.2% necessitate a careful balancing of the minimum carbon plus phosphorus and nickel plus manganese contents to assure this minimum age hardenability. Thus, it will be seen from the data for bars 4488—4495, at the bottom of Table II, that if the carbon plus phosphorus totals at least 0.45%, together with a nickel plus manganese total of at least 12%, the steel will age harden to upwards of "C" 32 Rockwell. On the other hand, if these requirements are not met for the analyses containing less than 0.3% carbon, the steel will not harden to the required minimum of "C" 32 Rockwell, as evidenced by reference to the results for bars 3900 and 3965 of Table II. With carbon upwards of 0.3%, the minimum nickel

60 Furthermore, whereas with the low phosphorus steels of the copending application it is necessary to cool rapidly as in a water quench from the solution temperature in order that the desired hardness may be attained in the steel after it is aged, we have found that when phosphorus over about 0.15% is present in the steel, the desired hardness over "C" 32 Rockwell may be attained in the steel after aging even though the cooling rate from the solution temperature is somewhat retarded as in an oil quench, or even an air cool of sections under about 1 inch thick. This obviously is of considerable advantage in the heat treatment of large sections which would suffer much less distortion when quenched in oil than when quenched in water.

70 The effect on age hardenability of varying chromium contents of the steel of the invention is shown by the following Table VI:

5  
*Table VI*

EFFECT OF CHROMIUM ON ATTAINABLE HARDNESS OF  
AUSTENITIC C-Mn-Ni-Cr STEELS CONTAINING PHOS-  
PHORUS  
[All specimens solution treated at 2150° F., water quenched, and aged at  
1300° F. for 16 hours.]

| Bar  | Analysis Percent—Balance Fe |     |     |     |     |      | Rockwell "C"<br>Hardness |                                 |
|------|-----------------------------|-----|-----|-----|-----|------|--------------------------|---------------------------------|
|      | C                           | Mn  | P   | Si  | Ni  | Cr   | As Quenched              | Aged at<br>1,300° F.<br>16 Hrs. |
| 4353 | .36                         | 3.5 | .27 | .36 | 8.8 | 0.7  | 23M                      | 22M                             |
| 4354 | .33                         | 3.6 | .29 | .34 | 9.3 | 4.9  | 4                        | 18                              |
| 4355 | .37                         | 3.6 | .29 | .49 | 9.3 | 9.8  | 11                       | 36                              |
| 4356 | .35                         | 3.7 | .29 | .48 | 9.0 | 12.8 | 13                       | 40                              |
| 4357 | .36                         | 3.4 | .29 | .45 | 9.3 | 14.0 | 13                       | 40                              |
| 4358 | .39                         | 3.4 | .28 | .49 | 9.4 | 16.4 | 15                       | 43                              |
| 4359 | .41                         | 3.4 | .29 | .34 | 9.3 | 17.8 | 14                       | 44                              |

M—magnetic; all others non-magnetic.

As shown by the above data, the chromium content must be at least about 10% in order to impart the minimum

## 6

a stable austenitic structure substantially free of ferrite.

When the steel is to be used under high stress at elevated temperature we generally include up to about 3% of either one or both of the carbine forming elements molybdenum and tungsten.

Nitrogen is generally over .03% in the steel of the invention and may be present up to about 0.40%.

Since the steel may be machined in the hardened condition after final heat treatment, we may include sulfur in the steel composition up to about 0.30% to improve machinability.

We may use different proportions of the elements carbon, manganese, phosphorus, silicon, nickel, chromium, molybdenum (or tungsten), and nitrogen in the steel de-

15 pending on the application. For an application requiring a non-magnetic material with high room temperature strength and good ductility, we generally balance the composition so that the carbon is on the low side of the range and nickel is present in larger amounts than manganese. Data on some compositions suitable for such an application are given in Table VII.

## Table VII

MECHANICAL AND PERMEABILITY PROPERTIES OF STEELS FOR NON-MAGNETIC HIGH STRENGTH APPLICATION

| Bar  | Analysis Percent—Balance Fe |     |     |     |      |      |     |
|------|-----------------------------|-----|-----|-----|------|------|-----|
|      | C                           | Mn  | P   | Si  | Ni   | Cr   | N   |
| 3941 | .36                         | 3.5 | .24 | .33 | 9.4  | 18.6 | .05 |
| 3942 | .34                         | 3.5 | .37 | .44 | 9.3  | 19.0 | .04 |
| 3944 | .51                         | 3.5 | .25 | .38 | 9.2  | 18.6 | .06 |
| 3945 | .46                         | 3.4 | .39 | .30 | 9.3  | 18.5 | .09 |
| 3947 | .36                         | 1.4 | .24 | .22 | 13.0 | 18.8 | .04 |
| 3948 | .33                         | 1.4 | .37 | .30 | 13.1 | 19.0 | .05 |
| 3950 | .49                         | 1.4 | .23 | .20 | 13.1 | 18.8 | .05 |
| 3951 | .47                         | 1.3 | .37 | .22 | 13.1 | 19.1 | .14 |

[Pieces in  $\frac{1}{8}$  sq. section solution treated as indicated; aged at 1300° F. for 16 hours; and machined to tensile, impact, and permeability test pieces.]

| Bar  | Solution Treat-<br>ment | "C"<br>Rock.<br>Hard. | 0.2%<br>Yield,<br>P. S. I. | Tensile<br>Strength,<br>P. S. I. | Elong.<br>in 1.4<br>in.,<br>Percent | Red.<br>Area,<br>Percent | V-Notch<br>Izod,<br>Ft.-Lbs. | Permea-<br>bility,<br>H=500 |
|------|-------------------------|-----------------------|----------------------------|----------------------------------|-------------------------------------|--------------------------|------------------------------|-----------------------------|
| 3941 | 2,050° F. water         | 34                    | 88,000                     | 146,000                          | 27.9                                | 37.5                     | -----                        | -----                       |
| 3941 | 2,150° F. water         | 38                    | 116,000                    | 167,000                          | 17.6                                | 26.5                     | -----                        | -----                       |
| 3942 | 1,950° F. water         | 36                    | 106,000                    | 155,000                          | 22.2                                | 33.5                     | 14                           | 1.003                       |
| 3942 | 1,950° F. air           | 35                    | 100,000                    | 152,000                          | 24.4                                | 29.0                     | 13                           | 1.002                       |
| 3942 | 2,050° F. water         | 41                    | 132,000                    | 175,000                          | 15.0                                | 24.5                     | -----                        | -----                       |
| 3944 | 2,050° F. water         | 33                    | 88,000                     | 149,000                          | 24.7                                | 33.0                     | -----                        | -----                       |
| 3944 | 2,150° F. water         | 42                    | 126,000                    | 177,000                          | 18.4                                | 25.0                     | -----                        | -----                       |
| 3945 | 1,950° F. water         | 40                    | 121,000                    | 167,000                          | 18.1                                | 27.0                     | 7                            | 1.003                       |
| 3945 | 1,950° F. air           | 39                    | 109,000                    | 160,000                          | 20.7                                | 26.0                     | 6                            | 1.003                       |
| 3947 | 2,150° F. water         | 35                    | 105,000                    | 155,000                          | 23.0                                | 33.5                     | 18                           | 1.003                       |
| 3947 | 2,150° F. air           | 35                    | 107,000                    | 153,000                          | 17.2                                | 29.5                     | 11                           | 1.003                       |
| 3947 | 2,200° F. water         | 39                    | 128,000                    | 171,000                          | 11.5                                | 15.5                     | -----                        | -----                       |
| 3948 | 1,950° F. water         | 33                    | 100,000                    | 145,000                          | 22.9                                | 41.5                     | -----                        | -----                       |
| 3948 | 2,050° F. water         | 39                    | 124,000                    | 166,000                          | 21.5                                | 35.5                     | 12                           | 1.003                       |
| 3950 | 2,150° F. water         | 36                    | 103,000                    | 155,000                          | 19.4                                | 30.0                     | 12                           | 1.003                       |
| 3950 | 2,150° F. air           | 36                    | 105,000                    | 155,000                          | 21.0                                | 29.0                     | 8                            | 1.002                       |
| 3951 | 1,950° F. water         | 34                    | 104,000                    | 149,000                          | 18.6                                | 30.5                     | -----                        | -----                       |
| 3951 | 1,950° F. air           | 33                    | 92,000                     | 143,000                          | 22.7                                | 30.0                     | -----                        | -----                       |
| 3951 | 2,050° F. water         | 40                    | 125,000                    | 166,000                          | 17.1                                | 28.5                     | 8                            | 1.003                       |

required age hardenability of "C" 32 Rockwell. The 60 preferred lower limit for the chromium content is about 12%, as the steels of the invention containing upwards of 12% chromium are found to be less brittle in the age hardened condition than those containing lesser chromium contents. An upper limit of 30% is set for the chromium range in order to assure retention of adequate forging characteristics of the alloy in the prehardened state.

Silicon is always present in the steel for deoxidation purposes and may be present up to about 3% for improving the resistance of the steel to oxidation at elevated 70 temperatures.

Chromium is present in our steel from about 10 to 30% to provide corrosion and oxidation resistance. As the chromium is increased, we generally increase also the sum of manganese and nickel so that the steel will have 75

The low permeability steels of the foregoing type having good forging and age hardening characteristics together with high strength, have the following preferred range of analysis: carbon about 0.2 to 0.5%; phosphorus about 0.2 to 0.4%, the sum of carbon and phosphorus being at least 0.45%; manganese about 1 to 5%, nickel about 8 to 15%, the sum of nickel and manganese being at least about 12%; chromium about 17 to 25%; silicon up to about 1%; nitrogen up to about 0.3%; sulfur up to about 0.3%; balance substantially all iron.

For steel to be used for automotive exhaust valves and similar parts, we generally balance the composition with carbon in the middle of the range and manganese in larger amount than nickel, although we may also use a high percentage of nickel as shown in the analysis of bar 4123 in the table below.

7  
Table VIII

## PROPERTIES OF STEELS SUITABLE FOR EXHAUST VALVE SERVICE

| Bar  | Analysis Percent—Bal. Fe |     |     |      |      |      |     | "C" Rock.<br>Sol. Treated:<br>2,150 °F.,<br>Aged:<br>1,300 °F., hrs. | Weight Loss<br>in 1 hr.:<br>Lead Oxide<br>at 1,675 °F.,<br>gms./sq.in. |
|------|--------------------------|-----|-----|------|------|------|-----|----------------------------------------------------------------------|------------------------------------------------------------------------|
|      | C                        | Mn  | P   | Si   | Ni   | Cr   | N   |                                                                      |                                                                        |
| 3817 | .60                      | 4.7 | .20 | .50  | 3.8  | 21.2 | .04 | 41                                                                   | 3.1                                                                    |
| 3975 | .36                      | 5.0 | .21 | .58  | 3.8  | 21.0 | .17 | 42                                                                   | 2.8                                                                    |
| 4116 | .46                      | 8.2 | .25 | .79  | 4.3  | 21.9 | .22 | 46                                                                   | 2.6                                                                    |
| 3978 | .56                      | 9.0 | .21 | .90  | 3.7  | 20.6 | .21 | 45                                                                   | 2.6                                                                    |
| 4118 | .44                      | 8.3 | .24 | 1.89 | 4.3  | 22.0 | .22 | 46                                                                   | 2.3                                                                    |
| 4120 | .45                      | 8.4 | .24 | 2.90 | 4.3  | 22.2 | .20 | 46                                                                   | 2.3                                                                    |
| 4123 | .53                      | 8.3 | .22 | .53  | 15.6 | 30.0 | .39 | 42                                                                   | 2.4                                                                    |
| 3820 | .60                      | 5.0 | .42 | .35  | 3.9  | 20.7 | .15 | 48                                                                   | 3.2                                                                    |

Steels of the foregoing type which are age hardenable to a minimum of "C" 38 Rockwell on solution treating at a temperature no higher than 2200° F., and subsequent aging at about 1300° F., have the following preferred range of analysis: Carbon about 0.4 to 0.7%; phosphorus about 0.15 to 0.45%; manganese about 1 to 12%; nickel about 3 to 25%, the sum of manganese and nickel being from about 9 to 30%; chromium from about 20 to 30%; silicon up to about 3%; nitrogen up to about 0.4%; sulfur up to about 0.3%; metal of the group molybdenum and tungsten up to about 3%; balance substantially iron.

For applications where strength at high temperatures for long time service is required, we generally include molybdenum (or tungsten) in the composition as stated above. Some data on steels suitable for high temperature applications such as steam power plant and gas turbine parts are given in Table IX.

Table IX

## PROPERTIES OF STEEL SUITABLE FOR SERVICE AT 1200° F. UNDER STRESS

| Bar  | Analysis Percent—Balance Fe |     |     |     |     |      |     |
|------|-----------------------------|-----|-----|-----|-----|------|-----|
|      | C                           | Mn  | P   | Si  | Ni  | Cr   | Mo  |
| 3933 | .51                         | 7.5 | .23 | .47 | 7.4 | 22.2 | 1.8 |
| 3936 | .61                         | 7.5 | .22 | .42 | 7.3 | 22.0 | 1.9 |
| 3939 | .72                         | 7.6 | .26 | .45 | 7.3 | 22.8 | 1.8 |
| 3937 | .58                         | 7.5 | .43 | .38 | 7.5 | 21.2 | 1.6 |

## ROOM TEMPERATURE PROPERTIES

| Bar  | Heat Treatment <sup>1</sup> | "C" Rock. Hard. | 0.2% Yield Strength, p. s. i. | Tensile Strength, p. s. i. | Elong. in 1.4 in., Percent | Red. Area, Percent | V-Notch Izod, Ft.-Lbs. |
|------|-----------------------------|-----------------|-------------------------------|----------------------------|----------------------------|--------------------|------------------------|
| 3933 | BB                          | 35              | 98,000                        | 156,000                    | 18.6                       | 25.0               | 7                      |
| 3933 | BO                          | 32              | 81,000                        | 141,000                    | 27.1                       | 30.5               | 15                     |
| 3936 | BB                          | 36              | 98,000                        | 154,000                    | 21.4                       | 23.5               | 7                      |
| 3936 | BO                          | 33              | 77,000                        | 137,000                    | 26.6                       | 32.5               | 13                     |
| 3939 | BO                          | 33              | 80,000                        | 140,000                    | 22.6                       | 27.5               | 55                     |

Table IX—Continued

## STRESS RUPTURE PROPERTIES AT 1,200° F.

| Bar | Heat Treatment <sup>1</sup> | Stress, p. s. i. | Rupture Time, Hours | Elongation, Percent in 1.4 in. | Percent Reduction Area |
|-----|-----------------------------|------------------|---------------------|--------------------------------|------------------------|
| 25  | BB                          | 56,000           | 89                  | 11.4                           | 20.0                   |
|     | BB                          | 62,000           | 119                 |                                |                        |
|     | BO                          | 56,000           | 203                 | 5.7                            | 15.0                   |
|     | BB                          | 56,000           | 82                  | 15.4                           | 27.0                   |
|     | BB                          | 62,000           | 196                 |                                |                        |
|     | BO                          | 56,000           | 184                 | 16.3                           | 20.0                   |
| 30  | BO                          | 62,000           | 197                 |                                |                        |
|     | BB                          | 56,000           | 85                  | 15.4                           | 21.5                   |
|     | BO                          | 56,000           | 96                  | 20.7                           | 27.5                   |
|     | BB                          | 62,000           | 204                 |                                |                        |
|     | BO                          | 56,000           | 527                 | 3.8                            | 8.5                    |

<sup>1</sup> Heat treatments: BB—2150° F., water quench; aged 1500° F.—16 hours. BO—2150° F., water quench; aged 1300° F.—16 hours; plus 1700° F.—2 hours.

<sup>2</sup> NOTE.—Test piece with 60 degree V-notch, diameter base of notch .252 in. with gage section .357 in. diameter; .005 in. radius base of notch.

40 A preferred range of analysis for steels of this type is: carbon about 0.45 to 0.7%; phosphorus about 0.2 to 0.45%; manganese about 5 to 12%; nickel about 4 to 18%; chromium about 20 to 30%; silicon up to about 3%; metal of the group molybdenum and tungsten, about 1 to 3%; nitrogen up to about 0.4%; sulfur up to about 0.3%; balance substantially iron.

45 It is of interest that the steels of this invention are quite resistant to overaging. Although the optimum aging temperature for maximum hardness is about 1250°/1300° F. good hardness is developed with aging temperatures as high as 1500° F. Furthermore, steel which has been aged at 1300° F. can be reheated for a short time at temperatures as high as 1700° F. without suffering much loss of hardness. Some data on the resistance of the steels of this invention to softening at high temperatures are shown in Table X.

Table X

## EFFECT OF HIGH TEMPERATURE HEATING ON HARDNESS OF C-Mn-P-Ni-Cr STEELS

[Specimens solution treated at 2150° F., water quenched, and aged as indicated.]

| Bar  | Analysis Percent—Balance Fe |     |     |     |     |      |     | "C" Rockwell Hardness |                           |                           |                           |                          |
|------|-----------------------------|-----|-----|-----|-----|------|-----|-----------------------|---------------------------|---------------------------|---------------------------|--------------------------|
|      | C                           | Mn  | P   | Si  | Ni  | Cr   | Mo  | As Q                  | Aged, 1,300° F., 16 hours | Aged, 1,400° F., 16 hours | Aged, 1,500° F., 16 hours | Aged, 1,700° F., 2 hours |
| 3933 | .51                         | 7.5 | .23 | .47 | 7.4 | 22.2 | 1.8 | 23                    | 40                        | 35                        | 33                        | 32                       |
| 3936 | .61                         | 7.5 | .22 | .42 | 7.3 | 22.0 | 1.9 | 24                    | 41                        | 35                        | 34                        | 33                       |
| 3939 | .72                         | 7.6 | .26 | .45 | 7.3 | 22.8 | 1.8 | 27                    | 41                        | 37                        | 34                        | 33                       |
| 3934 | .53                         | 7.5 | .41 | .36 | 7.3 | 21.5 | 1.7 | 24                    | 46                        | 42                        | 40                        | 39                       |
| 3937 | .58                         | 7.5 | .43 | .38 | 7.5 | 21.2 | 1.6 | 25                    | 46                        | 43                        | 38                        | 39                       |

What we claim is:

1. Age hardenable austenitic steel characterized in being hardenable to a minimum of about "C" 32 Rockwell after solution treatment at a temperature no higher than 2200° F. and subsequent aging at about 1300° F. for about 15 hours, said steel consisting essentially of about: 0.2 to less than 0.3% carbon and 0.15 to 1% phosphorus, the sum of carbon and phosphorus being at least 0.45%; 0.5 to 15% manganese; 5 3 to 25% nickel, the sum of nickel and manganese being about 12 to 30%; 10 10 to 30% chromium; up to about 3% silicon; up to about 3% of metal selected from the group consisting of molybdenum and tungsten; up to about 0.4% nitrogen; up to about 0.3% sulfur; and the balance iron.

2. A precipitation hardened, austenitic alloy steel, hav- 15

ing a hardness of at least "C" 32 Rockwell, said steel consisting essentially of about: 0.2 to less than 0.3% carbon and 0.15 to 1% phosphorus, the sum of carbon and phosphorus being at least 0.45%; 0.5 to 15% manganese; 5 3 to 25% nickel, the sum of nickel and manganese being about 12 to 30%; 10 to 30% chromium; up to about 3% silicon; up to about 3% of metal selected from the group consisting of molybdenum and tungsten; up to about 0.4% nitrogen; up to about 0.3% sulfur; and the balance iron.

References Cited in the file of this patent

UNITED STATES PATENTS

|           |                |                |
|-----------|----------------|----------------|
| 2,523,917 | Payson         | Sept. 26, 1950 |
| 2,528,637 | Clarke         | Nov. 7, 1950   |
| 2,686,116 | Schempp et al. | Aug. 10, 1954  |